

## UNITED STATES PATENT OFFICE

JUDSON A. DE CEW, OF MOUNT VERNON, NEW YORK, ASSIGNOR TO PROCESS ENGINEERS, INC., OF NEW YORK, N. Y., A CORPORATION OF NEW YORK

METHOD OF TREATING WOOD PULP FIBERS AND PAPER PRODUCT MADE THEREFROM

No Drawing. Application filed September 19, 1929, Serial No. 393,845, and in Canada February 14, 1929.

In the manufacture of newsprint paper, which consists essentially of a mixture of ground wood and sulphite pulp formed into a sheet of paper, there is an important manufacturing problem resulting from the tendency of these pulps to stick to presses and wires of the paper machine because of certain resinous material in the pulps. When this happens, the pitch coming from these pulps accumulates on the moving wires and it is necessary to close down the machine and clean the wires by hand labor, resulting in considerable expense and loss of production.

Wood that is used for newsprint pulp often contains various proportions of balsam or jack pine mixed with the spruce and these woods contain a considerable quantity of resinous material. Spruce contains less resin than any other wood that is used for the manufacture of newsprint but sometimes this contains enough resinous material to cause difficulty. Jack pine is a wood which could be used in the manufacture of newsprint if the resins could be dissolved in the sulphite process or if the pulp made from it without removing the resins could be used mechanically in the manufacture of paper. The resinous material is not injurious to the paper but is an ingredient which causes difficulty in the manufacturing process.

Sulphite pulp from such wood will contain portions of this resinous material in a globular form and a portion of this washes out of the pulp and onto the paper machine clothing (consisting of felts and wires) and sticks to these fabrics.

Ground wood made from fresh wood also contains sticky resinous material. Many methods have been tried to remove this trouble but as long as the woods carry variable quantities of this resin, the trouble is likely to reoccur regularly in many mills.

The pitchy matter found in ground wood or sulphite pulp does not act as a sizing agent even if it is present in sufficient quantity to cause great difficulty on the machine because it is not like a hydrated precipitate of rosin, but is in the form of globules with no covering power, but which adhere to the surface of the fibers in spots.

The problem to solve in making newsprint paper is to change the resinous globules from a condition that is adhesive to one that is not adhesive, and at the same time to produce a paper that would not be classified as a sized paper. In order to accomplish this I use a lubricating emulsion of wax or oil which will surround or cover the resinous globules so that they will not adhere to the fabric of the paper machine. If these emulsions are not coagulated in any way they will be mostly washed away through the paper machine wire, but by surrounding the pitchy material they will keep it from sticking to the various parts of the machine. This is the most desirable method of operating unless machine conditions make it necessary to use some coagulant. By dilution and agitation, a portion of the emulsion will be fixed on the resinous fibers without any coagulant. There will be no objection to coagulating these emulsions and retaining more of them in the paper if this can be done without coating the fibers in such a way as to produce a sized paper. In my United States Patent No. 1,317,618 I have described a paper product that is made water proof by precipitating an emulsion of rosin and wax on the paper fibers. In my United States Patent No. 1,174,697, I described an emulsion made from rosin and wax, which had first been blended together and then emulsified. In these patents and in all other methods where wax emulsions may have been used in conjunction with pulp fibers, the purpose and result of such application has been the production of a sized or water proof product.

My present invention differs from these owing to the fact that I now use a wax emulsion, that will coat or surround the natural resinous globules with pulp but the wax is not permanently emulsified with such resin, or blended with it by solution and consequently an entirely different result is obtained by this process than any that has been used heretofore.

It is well recognized in the art of sizing paper that sulphate of alumina, called "alum", is an essential ingredient in paper making. It is the accompanying sizing in-

gredient that is necessary to use as a coagulant in order to produce a sized paper. Its use produces a slightly acid reaction which makes the sizing water repellent, whereas, if the sizing remains neutral or slightly alkaline it is not water repellent. The same applies to the paper fibers so that when alum is not used a sized paper is not produced.

In order to use wax emulsions as a lubricant and not a sizing material, it is only necessary to discard the use of sulphate of alumina.

It is not material to the application of my process whether the lubricating emulsions are coagulated or not except that if they should be coagulated by any neutral or alkaline salts that may be present in the stock, it will only reduce the amount of emulsion lost in the waste water, and will not produce a sized paper. I may even add a calcium or other neutral salt in order to fix the emulsion on the resinous water.

As an example of the manner in which my process may be carried out, I mix with the batch of pulp fibers an amount of emulsified waxy material, which is approximately equal to the amount of resinous or pitchy material contained in the fibers. This is generally sufficient to cover the resinous particles so that the portion that comes in contact with the paper machine wire or felt will wash away without sticking to it.

For ordinary spruce wood, one-half of 1% of wax will be sufficient to accomplish this result but for very pitchy wood more may be necessary.

Standard newsprint is an unsized paper although some small amounts of rosin size and alum may be used to improve the finish and retain the fine fibers. Rosin size tends to make the fibers stick to the machine whereas alum has a tendency to remove this sticking. Alum has a corroding effect upon the machine and piping of the mill and does considerable damage but it is used because no better means is known to get the paper over the machine at the highest speed with the fewest breaks.

A method that will enable the paper mill to make a neutral or alkaline paper at the highest possible speed will be of great benefit to the makers of newsprint paper.

If I coagulate the amount of lubricating emulsion with which I cover the pitch, by using a neutral salt of calcium or magnesian or any other neutral salt, the finish of paper will be improved and the fine fibers retained but the paper will not be water repellent or sized.

I may use wax or oil emulsions that are either alkaline or neutral and which may be made by any process of emulsification, my invention not being in the method of making wax emulsions but in the method of applying them for a new purpose to produce a new re-

sult, namely an unsized paper containing wax as a lubricant, covering the resinous matter in the paper.

While many modifications may be made in carrying out my process, the scope of this invention is intended to cover the use of wax or oil or other lubricating emulsions mixed with paper pulp in a neutral or alkaline condition and either dispersed or coagulated for the purpose of removing the sticky properties of said pulp. The emulsions may be used in any proportion sufficient to remove any stickiness as long as a sized paper is not produced.

This process is particularly adapted to the manufacture of standard newsprint, the specifications and limitations of which are well known, especially with respect to sizing.

Having now described the invention, what is claimed as new, and for which Letters Patent of the United States is desired, is:

1. A method of making standard newsprint paper which consists in covering the natural resins in the pulp with an emulsion of waxy material.

2. A step in the manufacture of standard newsprint paper which consists in adding a non-sizing lubrication emulsion to the pulp stock while the paper is in process of manufacture.

3. A step in the manufacture of newsprint paper which consists in adding sufficient lubricating emulsion to the pulp stock to keep it from sticking to the paper machines and making therefrom a sheet of unsized paper.

4. A step in the manufacture of paper which consists in adding a lubricating emulsion to the pulp stock and coagulating the emulsion with a salt that will produce an unsized paper.

5. A step in the manufacture of paper which consists in coagulating a wax emulsion in the pulp fibers, with an alkaline salt, and producing an unsized paper.

6. A method of producing an unsized paper containing wax surrounding the natural resins, which consists in coagulating an emulsion containing wax in the pulp by means of an earth salt.

7. A method of treating the natural resinous material in pulp fibers, which consists in depositing over said resins from an emulsion, a non-sizing lubricant.

8. A method of preventing the natural resins in paper pulp from sticking to the paper machine, which consists in surrounding these resins with an emulsified wax composition without subsequent coagulation by alum.

9. A method of treating the natural resins in a paper pulp which consists in adding to the pulp an amount of waxy emulsion approximately equal to the amount of resins.

10. A method of making an unsized paper containing wax which consists in adding a

wax emulsion to the paper which will be dispersed and partly coagulated by dilution.

11. A paper product having a non-sizing lubricant coagulated over the surface of its 5 natural resins.

12. An unsized paper product having its resinous impurities coated with a waxy material.

13. An alkaline newsprint paper, the paper 10 stock of which has been treated with an alkaline lubricating emulsion during the process of manufacture.

14. A natural newsprint paper which has been treated in the manufacturing process 15 with a natural lubricating emulsion.

15. A paper product containing an amount of waxy lubricant approximately equal to the amount of natural resins in the fiber.

Signed at New York, in the county of Nassau and State of New York, this 17th day of 20 September, 1929.

JUDSON A. DE CEW.